

**1**

3,730,911

**HEATING ELEMENT COMPRISING LANTHANUM CHROMITE AND OXIDATION-RESISTANT SILICON COMPOUND**

Gérard Aubin, Evreux, and David Yerouchalmi, Le Mesnil Saint-Denis, France, assignors to Commissariat à l'Energie Atomique, Paris, France  
No Drawing. Filed Oct. 4, 1971, Ser. No. 186,425  
Claims priority, application France, Oct. 5, 1970,

7035867

Int. Cl. H01b 1/06

U.S. Cl. 252—516

**1 Claim****ABSTRACT OF THE DISCLOSURE**

A heating element which is electrically conductive from room temperature to at least 2000° C. in an oxidizing atmosphere and over a long period of time, the element being formed from a lanthanide chromite which is combined with a variable proportion of an oxidation-resistant silicon compound.

This invention relates to a heating element in which the production of heat is obtained by Joule effect resulting from the flow of an electric current, said element being capable of operating within a range extending from room temperature to temperatures above 2000° C. and even more especially in an oxidizing atmosphere.

Among the known applications of electrically conductive heating elements, the most noteworthy are those which are designed in the form of wires, cables, strips, plates, deposits and the like which are fabricated from metals such as molybdenum, tantalum, niobium, tungsten or from a metalloid such as graphite. These elements permit of satisfactory operation from room temperature to temperatures which can attain 2500 or even 3000° C. provided that work is carried out in a neutral atmosphere over a period of time which does not exceed approximately twenty hours. Consideration has also been given to the fabrication of heating elements from a compound such as silicon carbide which is formed by means of special binders and permits of satisfactory operation in time and in an oxidizing atmosphere but only on condition that the temperature does not exceed 1600° C. Other compounds such as molybdenum alloyed with a given percentage of molybdenum silicide permit of operation up to a maximum temperature of 1750° C. with a certain degree of safety. Finally, it has already been proposed to make use of certain refractory oxides and especially lime-stabilized zirconium oxide, yttrium oxide, magnesia or different rare earths or thorium oxide (thoria). There is also a major drawback to be taken into consideration in this case since refractory oxides of this type are electrically conductive only after preheating to approximately 1200° C. This does not permit continuous operation of the heating element above room temperature and entails the need for more conventional ancillary circuits which call for protection as soon as the temperature reaches the threshold value of 1200° C. at which the element proper comes into operation.

An appreciable advance in the technology of electrically conductive heating elements has consisted in employing as constituent material of said element either chromium oxide combined with alumina or alternatively chromites of lanthanides which may be mixed with zirconia if necessary, the function of these compounds being to permit the flow of electric current from room temperature upwards when they are produced in the form of solids having very high density (87 to 99% of theoretical), in which case their electrical conductivity is of the order of 40 to 120 mhos/meter. Unfortunately, these

**2**

compounds have relatively high vapor pressures as soon as the temperature exceeds 1600° C., particularly in an oxidizing atmosphere in which the measured evaporation rate is approximately one hundred times higher than in a neutral atmosphere and especially an argon atmosphere. This even holds true in the case of the most refractory and the most highly conductive chromite, namely lanthanum chromite which has a melting point of approximately 2450° C., although the addition of zirconia does have a beneficial effect in limiting to a certain extent the evaporation of the chromite which combines partially with the zirconia under the conditions of use which have been mentioned in the foregoing. Moreover, these different compounds have relatively low thermal conduction and are thus very delicate by reason of the thermomechanical stresses and especially thermal shocks to which they are subjected when the temperature rises. If these compounds remain acceptable for use in spite of their high vapor pressure in an oxidizing atmosphere which results in rapid wear, it is in that case necessary to take very strict precautions when initiating either an increase or decrease in temperature; moreover, it is practically essential to fabricate the heating elements in the form of conductors having a very small cross-sectional area. These different factors make it difficult to employ these heating elements in practice and result in capital costs which are usually of a very high order.

The present invention overcomes the disadvantages of the various solutions which have been proposed heretofore by means of a heating element which is conductive from room temperature up to temperatures of at least 2000° C. and permits utilization in an oxidizing atmosphere over very long periods of time.

To this end, the invention consists in fabricating the heating element from a chromite of the lanthanide series combined with a variable proportion of at least one silicon compound which exhibits oxidation resistance.

According to one preferred feature, the chromite of the lanthanide series is lanthanum chromite whilst the silicon compound can be selected from molybdenum silicon  $MoSi_2$ , silicon nitride  $Si_3N_4$ , silicon carbide  $SiC$  or a mixture of zirconium boride  $ZrB_2$  and molybdenum silicide  $MoSi_2$ .

According to another preferred feature, the variable proportion of the silicon compound is within the range of 5 to 20% by weight.

The invention therefore consists in combining with a highly refractory compound such as a chromite of the lanthanide series of elements and especially lanthanum chromite which is electrically conductive from room temperature to at least 2000° C. a suitable silicon compound whose intended functions are to reduce to a considerable extent the vapor pressure of the chromite which is employed in particular in an oxidizing atmosphere, to increase the thermal conduction of the chromite and therefore to make this latter less sensitive to thermal shocks without thereby modifying its oxidation resistance. The silicon compound is chosen so as to ensure that, during the process of manufacture, the grains of the chromite which is employed are coated with a refractory silica film which prevents vaporization of the chromite and isolates this latter from the surrounding atmosphere which can especially be highly oxidizing. The heating element thus formed can be produced with equal ease in the form of bars, strips, rods, hairpin elements, plates, cylinders and the like while being suited in each case to a particular use and especially for furnaces of the tubular or parallel-epipedal type employed in industrial laboratories, the susceptors of high-frequency circuits or alternatively other thermal applications involving either intermittent or continuous operation.

The advantages of the heating elements which are produced in accordance with the invention are essentially as follows: these elements are electrically conductive from room temperature to a temperature which is higher than 2000° C. and consequently dispense with the need for ancillary circuits in furnaces or the like having either zirconium or thorium oxide elements in which the use of the heating element can be contemplated only at temperatures above 1100 to 1200° C.; these ancillary circuits are usually formed of silicon carbide and have to be protected above this threshold value in order to prevent melting. The heating elements of lanthanide chromite alloyed with a silicon compound can also readily be employed in an oxidizing atmosphere (also, of course, in a neutral atmosphere) for any length of time which may be necessary. Finally, the operation of the elements can be maintained at the maximum temperature during these periods of time without any difficulty.

By way of indication, the manufacture of a heating element in accordance with the invention involves the following steps: in a first step, the manufacture of lanthanum chromite is carried out in a solar or plasma furnace starting from chromium oxide and lanthanum oxide which are mixed in stoichiometric proportions. The product obtained is then ground to a powder having a particle size between 1 and 5 microns to which is added in adequate proportions within the range of 5 to 20% a silicon compound which is preferably selected from the products referred to earlier. The mixture which is thus formed is then finally shaped in a mold within an isostatic press under a pressure within the range of 1.5 to 5 t./cm.<sup>2</sup> in order to obtain a part having a density which varies between 90 and 95% of theoretical. The final step consists in carrying out a baking process within a gas furnace in a slightly oxidizing

atmosphere with a level-temperature stage at 1650-1700° C. for a period of one to two hours; during this step, the partial conversion of the silicon compound to silica results in coating of the lanthanum chromite grains. Heating tests are then carried out with a temperature rise in successive stages of 100 to 200° C. per hour with a longer stage at 1600° C.

It must clearly be understood that the invention is not limited in any sense to the examples which have been more especially contemplated in the foregoing but extends on the contrary to all alternative forms.

What we claim is:

1. A heating element having reduced vapor pressure and improved thermal conductivity and electrically conductive from room temperature to at least 2000° C. in an oxidizing atmosphere and over a long period of operation comprising a mixture of lanthanum chromite and from 5 to 20% by weight of at least one oxidation-resistant silicon compound selected from the group consisting of molybdenum silicide, silicon nitride, silicon carbide and a mixture of molybdenum silicide and zirconium boride.

#### References Cited

#### UNITED STATES PATENTS

|    |           |         |                      |           |
|----|-----------|---------|----------------------|-----------|
| 25 | 3,475,352 | 10/1969 | Anthony et al. _____ | 252—521 X |
|    | 3,531,421 | 9/1970  | Foex et al. _____    | 252—521 X |
|    | 3,321,727 | 5/1967  | Schrevelius _____    | 252—516 X |
|    | 3,171,871 | 3/1965  | Watson et al. _____  | 252—516 X |
| 30 | 3,490,067 | 1/1970  | Foex _____           | 252—521   |

CHARLES E. VAN HORN, Primary Examiner

U.S. Cl. X.R.

252—518, 521; 219—553